

## UNITED STATES PATENT OFFICE

JAMES ASTON AND ADDISON H. BEALE, OF PITTSBURGH, PENNSYLVANIA, ASSIGNEES,  
BY MESNE ASSIGNMENTS, TO A. M. BYERS COMPANY, OF PITTSBURGH, PENNSYLVANIA,  
A CORPORATION OF PENNSYLVANIA

## MANUFACTURE OF WROUGHT IRON FROM BESSEMER STEEL

No Drawing.

Application filed July 19, 1928. Serial No. 294,049.

Our invention relates to the Aston process of making wrought iron, such, for example, as set forth in several United States patents of James Aston, such as No. 1,370,507, granted March 8, 1920, for Method of making wrought iron pipe; No. 1,412,823, granted April 18, 1922, for Method of making wrought iron; and No. 1,469,373, granted October 2, 1923, for Manufacture of wrought iron.

Our invention relates to the manufacture of wrought iron in accordance with the Aston process from Bessemer converter metal. It has been found in practice that the use of the Bessemer converter has certain advantages over the use of open hearth steel or electric steel. After considerable experimenting with Bessemer metal in the Aston process, we have discovered that the quality of the wrought iron ball produced in the Aston process is improved, and a better reaction obtained between the poured-in steel and the puddle slag when the converter heat is "full blown"—that is, when the carbon is reduced to below .10%. In practice we preferably blow the heat down to about .06%, which, in general steel practice, is termed a full or over-blown heat.

In Bessemer practice, it is well known that if such a heat were cast directly into ingots the product would be red short and would crack in working the same. For this reason, in Bessemer steel practice, deoxidizing agents, such as manganese, silicon and aluminum, are added, these elements, or combinations of them with similar elements, combining with the oxygen in the material to deoxidize and degasify the same.

We have discovered that in the Aston process when Bessemerized metal which is blown to such an extent that the carbon is below .10%, and preferably about .06%, is used, the oxidized condition of the steel, which would produce red shortness in the final material, is overcome by the deoxidizing and degasifying action of the bath of puddle slag into which the metal is poured for shotting. A reaction takes place between the blown metal and the iron oxide slag which causes deoxidation and degasification of the metal

during the shotting process in the slag. Consequently, the material rolled from the resulting ball formed in the lower part of the slag receptacle possesses the highest qualities of genuine hand puddled iron.

On the other hand, we have found that a heat that was blown "young" so that it contained above about .10% carbon, produced, when shotted in the same manner, a red short iron. We have also found that if the slag contains too high a percentage of silica, the full blown metal does not lose its red-shortness, and during the rolling process works in the manner of what the puddlers term "dry iron". That is, it does not have the desired welding qualities.

In practice we have found that in order to get a high quality of wrought iron ball, the content of silica in the slag should be less than about 15% and preferably not materially above 10%. Examples of such slags which we have used are as follows:

*Example I.*—A slag containing about 68.47% FeO, about 12.20% of  $Fe_2O_3$  and about 9.92% of  $SiO_2$ .

*Example II.*—A slag containing 72.13% of FeO, 7.26% of  $Fe_2O_3$  and 10.56% of  $SiO_2$ .

*Example III.*—A slag containing about 10.18% of  $SiO_2$ .

These slags usually contain a small percentage of phosphoric acid, manganous oxides, alumina and magnesia, but the essential constituents are those of the silica and iron oxides.

This process obviates the need of expensive and troublesome deoxidizers and degasifiers, makes the process capable of great regularity, and improves the product. The carrying out of the Bessemer operation to a point where the carbon is below .10% and down to a point of about .06%, is comparatively easy, and heat after heat may be made with great regularity. On the other hand, when carbon is present in larger percentages, we have found that it is liable to segregate and be un-uniformly distributed in the puddle ball, causing hard spots and failures in the finished product.

We have also found in the experimental

development, that the content of carbon and silicon combined in the steel when ready for pouring should be less than .20%, as this aids in reducing or substantially eliminating 5 red shortness in the wrought iron produced. The silicon should at least be below .09% in the metal to be shotted, and is preferably far below this. High silicon in steel tends to 10 make the material too "dry" and to interfere with the proper formation of the wrought iron ball.

We have also found in this connection that the percentage of oxygen in the steel as 15 poured should be less than about .31%, while the carbon and silicon together are less than .20%. In such case we have found that the addition of a deoxidizing metalloid or metalloids is unnecessary, although of course some small additions may be made, especially 20 if the metal is too "wild" for proper pouring, in order to partially "kill" the metal and bring it into better pouring condition for the shotting operation. In any case, if such metalloid additions are made to the steel before 25 pouring, they should not raise the combined content of carbon and silicon to over .20%. The manganese percentage should also be relatively low. All of these features, discovered during the experimental and development 30 period, have been found to be of advantage in obtaining the proper quality and uniformity of product.

The advantages of our invention result from the discovery that the carbon should be 35 blown to a point below .10% and preferably down to about .06%, and that when this is done deoxidizers are unnecessary, since the action of a proper puddle slag with the desirable percentage of iron oxides, such as 40 present in good puddle slag, will give an excellent product.

The slag should contain not over about 15% of silica, and preferably not materially above 10%, to give the best product. Additions 45 may be made to the blown metal, although this is not necessary.

Changes may be made in the Bessemer converter used, the metal may be side blown or bottom blown, although we prefer the bottom blow, and other variations may be made 50 without departing from our invention.

We claim:

1. In the manufacture of wrought iron, the steps consisting of Bessemerizing metal until 55 the carbon is below .10%, and then shotting the same in a bath of iron silicate puddle slag and forming a welded puddle-ball therein.
2. In the manufacture of wrought iron, the steps consisting of blowing metal to a "full blow", and then pouring the same into a bath of iron silicate puddle slag shotting the metal therein and forming a welded puddle-ball in the bath.
3. In the manufacture of wrought iron,

the steps consisting of blowing ferrous metal until the carbon content is about .06%, and then pouring the same into and shotting it in a bath of iron silicate slag and thereby deoxidizing and degasifying the same, and forming a welded ball at the bottom of the bath.

4. In the manufacture of wrought iron, the steps consisting of blowing a heat of steel to a "full blow", and then, without substantial additions, pouring the same into a bath of iron silicate slag and thereby deoxidizing and degasifying the same, and forming a welded puddle-ball therein.

5. In the manufacture of wrought iron, 80 the steps consisting of Bessemerizing metal until the carbon is below .10%, and then pouring the same into a bath of iron silicate slag having a silica content of not over about 15%, and forming a welded puddle-ball 85 therein.

6. In the manufacture of wrought iron, the steps consisting of Bessemerizing metal until the carbon is below .10%, and then pouring the same into a bath of iron silicate 90 slag having a silica content not materially over about 10%, and forming a welded puddle-ball therein.

7. In the manufacture of wrought iron, the steps consisting of granulating a molten steel 95 product wherein carbon and silicon taken together amount to less than about .20%, and mixing the same with a slag of puddling characteristics and forming a welded puddle-ball therewith.

8. In the manufacture of wrought iron, the steps consisting of forming a steel product by the Bessemer process wherein the carbon and silicon taken together are less than about .20%, granulating the same, and mixing the 105 granules while retaining at least a part of their original heat with a slag of puddling characteristics.

9. In the manufacture of wrought iron, the steps consisting of producing a molten 110 steel product containing carbon and silicon which, together, amount to less than about .20%, pouring the same into a slag bath of puddling characteristics, and granulating the same therein.

10. In the manufacture of wrought iron, the steps consisting of forming a steel product wherein the carbon and silicon taken together are less than .20%, and pouring said 120 steel product while molten into a slag bath of puddling characteristics to granulate it therein.

11. In the manufacture of wrought iron, the steps consisting of Bessemerizing molten iron, forming a molten steel product wherein the carbon and silicon taken together are less than .20%, and the oxygen content is less than .31%, granulating the same, and mixing the granulated product with a slag of 125 puddling characteristics.

12. In the manufacture of wrought iron, the steps consisting of Bessemerizing molten iron, forming a molten steel product wherein the carbon and silicon taken together are less than .20%, and the oxygen content is less than .31%, and pouring the same while molten into a slag bath of puddling characteristics.

13. In the manufacture of wrought iron, the steps consisting of forming a steel product with an oxygen content below about .31%, pouring the same into a slag bath of iron silicate character containing iron oxides, and absorbing the oxides from the metal into the slag as the comminuted or granulated metal descends through said slag.

14. In the manufacture of wrought iron, the steps consisting of forming a steel product containing carbon and silicon which together amount to less than .20%, and with an oxygen content below about .31%, pouring the same into a slag bath of iron silicate character containing iron oxides, and absorbing the oxides from the metal into the slag as the comminuted or granulated metal descends through the slag.

15. In the manufacture of wrought iron, the steps consisting of Bessemerizing metal until the carbon is about .06% and the silicon is less than .09%, pouring the molten steel product into a bath of iron silicate slag, granulating the same therein and forming a welded puddle-ball in the lower part of the bath.

16. In the manufacture of wrought iron, the step comprising pouring the product of a steel making operation into a molten bath of iron silicate slag having a silica content of not over about 13%.

40 In testimony whereof we have hereunto set our hands.

JAMES ASTON.  
ADDISON H. BEALE.

12. In the manufacture of wrought iron, the steps consisting of Bessemerizing molten iron, forming a molten steel product where in the carbon and silicon taken together are less than .20%, and the oxygen content is less than .31%, and pouring the same while molten into a slag bath of puddling characteristics.

13. In the manufacture of wrought iron, 10 the steps consisting of forming a steel product with an oxygen content below about .31%, pouring the same into a slag bath of iron silicate character containing iron oxides, and absorbing the oxides from the metal into the 15 slag as the comminuted or granulated metal descends through said slag.

14. In the manufacture of wrought iron, the steps consisting of forming a steel product containing carbon and silicon which together amount to less than .20%, and with 20 an oxygen content below about .31%, pouring the same into a slag bath of iron silicate character containing iron oxides, and absorbing the oxides from the metal into the slag 25 as the comminuted or granulated metal descends through the slag.

15. In the manufacture of wrought iron, the steps consisting of Bessemerizing metal until the carbon is about .06% and the silicon is less than .09%, pouring the molten steel product into a bath of iron silicate slag, 30 granulating the same therein and forming a welded puddle-ball in the lower part of the bath.

35 16. In the manufacture of wrought iron, the step comprising pouring the product of a steel making operation into a molten bath of iron silicate slag having a silica content of not over about 13%.

40 In testimony whereof we have hereunto set our hands.

JAMES ASTON.  
ADDISON H. BEALE.

#### Certificate of Correction

Patent No. 1,820,177.

Granted August 25, 1931, to

JAMES ASTON ET AL.

It is hereby certified that error appears in the printed specification of the above numbered patent requiring correction as follows: Page 1, lines 79 and 80, strike out "Example I.—A slag containing about 10.18% of  $SiO_2$ ." and insert instead 72.30% of  $FeO$  to 10.20% of  $Fe_2O_3$  and about 10.18% of  $SiO_2$ ; and that the said Letters Patent should be read with these corrections therein that the same may conform to the record of the case in the Patent Office.

Signed and sealed this 22nd day of September, A. D. 1931.

[SEAL.]

M. J. MOORE,  
Acting Commissioner of Patents.

**Certificate of Correction**

**Patent No. 1,820,177.**

**Granted August 25, 1931, to**

**JAMES ASTON ET AL.**

It is hereby certified that error appears in the printed specification of the above numbered patent requiring correction as follows: Page 1, lines 79 and 80, strike out "*Example 1.—A slag containing about 10.18% of SiO<sub>2</sub>.*" and insert instead *72.30% of FeO to 10.20% of Fe<sub>2</sub>O<sub>3</sub>, and about 10.18% of SiO<sub>2</sub>.*"; and that the said Letters Patent should be read with these corrections therein that the same may conform to the record of the case in the Patent Office.

Signed and sealed this 22nd day of September, A. D. 1931.

[**SEAL.**]

**M. J. MOORE,**  
*Acting Commissioner of Patents.*